



US006007974A

# United States Patent [19]

Begley et al.

[11] Patent Number: 6,007,974

[45] Date of Patent: \*Dec. 28, 1999

[54] SILVER HALIDE ELEMENT CONTAINING TRIAZOLE INHIBITORS

[75] Inventors: William J. Begley, Webster; Frank D. Coms; Teh-Hsuan Chen, both of Fairport; Donald Singleton, Jr., Olcott, all of N.Y.

[73] Assignee: Eastman Kodak Company, Rochester, N.Y.

[ \* ] Notice: This patent is subject to a terminal disclaimer.

[21] Appl. No.: 09/020,117

[22] Filed: Feb. 6, 1998

## Related U.S. Application Data

[63] Continuation-in-part of application No. 08/733,619, Oct. 17, 1996, abandoned.

[51] Int. Cl.<sup>6</sup> ..... G03C 1/08; G03C 7/26; G03C 7/32

[52] U.S. Cl. ..... 430/544; 430/553; 430/555; 430/557; 430/558; 430/955; 430/957

[58] Field of Search ..... 430/544, 553, 430/557, 555, 558, 957, 955

## References Cited

### U.S. PATENT DOCUMENTS

|           |         |                  |       |         |
|-----------|---------|------------------|-------|---------|
| 3,617,291 | 11/1971 | Sawdey           | ..... | 430/544 |
| 4,477,563 | 10/1984 | Ichijima et al.  | ..... | 430/544 |
| 5,356,764 | 10/1994 | Szajewski et al. | ..... | 430/505 |
| 5,759,757 | 6/1998  | Begley et al.    | ..... | 430/505 |

### FOREIGN PATENT DOCUMENTS

|           |         |                    |       |
|-----------|---------|--------------------|-------|
| 0 320 691 | 6/1989  | European Pat. Off. | ..... |
| 0 349 332 | 1/1990  | European Pat. Off. | ..... |
| 0 452 883 | 10/1991 | European Pat. Off. | ..... |
| 0 657 776 | 6/1995  | European Pat. Off. | ..... |
| 1382861   | 2/1975  | United Kingdom     | ..... |

## OTHER PUBLICATIONS

Patent Abstracts of Japan, vol. 012, No. 406 (P-777), Oct. 24, 1988 &amp; JP 63 144353 A, Jun. 16, 1988.

Primary Examiner—Geraldine Letscher  
Attorney, Agent, or Firm—Sarah Meeks Roberts

[57]

## ABSTRACT

This invention relates to a photographic element comprising a support having situated thereon at least one silver halide emulsion layer, the element further containing an image modifying coupler which upon reaction with oxidized color developing agent during processing forms a dye, said image modifying coupler represented by the formula



wherein

COUP is a photographic coupler moiety;

 $\text{T}^1$  is a timing or linking group; $\text{R}^1$  and  $\text{R}^2$  are independently selected from a halide atom, or an aliphatic, carbocyclic, heterocyclic, carbamoyl, sulfamoyl, carbonamido, sulfonamido, acyl, sulfo, nitro, cyano, amino, alkoxy, alkoxyalkyl, aryloxy, aryloxyalkyl, thioalkoxy, thioalkoxyalkyl, thioaryloxy, or thioaryloxyalkyl group; and $n$  is selected from 0, 1 or 2. More particularly this invention relates to a photographic element containing the above image modifying coupler wherein  $n$  is 0 and  $\text{R}^1$  and  $\text{R}^2$  are independently represented by the formula:\*\*—(Z)<sub>m</sub>—(X)<sub>r</sub>—R<sup>3</sup>\*\* point of attachment to triazole moiety  
wherein;

Z is an aliphatic, carbocyclic, or heterocyclic group.

**30 Claims, No Drawings**

# SILVER HALIDE ELEMENT CONTAINING TRIAZOLE INHIBITORS

## CROSS-REFERENCE TO RELATED APPLICATIONS

This is a continuation-in-part application of Ser. No. 08/733,619, filed Oct. 17, 1996, now abandoned entitled "Silver Halide Element Containing Triazole Inhibitors" by Begley et al.

## FIELD OF THE INVENTION

This invention relates to development inhibitor releasing couplers and silver halide photographic elements containing such couplers.

## BACKGROUND OF THE INVENTION

Various ways are recognized in the photographic industry for releasing a photographic inhibitor from a coupler in a photographic silver halide material and process. Release can be indirect through a linking or timing group or it can be direct, for example, upon reaction of the coupler with oxidized color developing agent during processing. Image-modifying couplers that release photographic inhibitors directly from the coupler are preferred in the photographic industry because manufacturing such couplers is easier, faster and less costly. However, many times direct release couplers, due to their inflexibility with regard to timing of release, are not practical for and effective at providing desired effects such as reduction of gradation, production of a finer color grain, improvement of sharpness through the so-called edge effect and improvement of color purity and color brilliance through inter-image effects. In this connection, reference is made to the article by C. R. Barr, J. R. Thirtle and P. W. Vittum entitled "Development-Inhibitor-Releasing (DIR) Couplers in Color Photography" in Photographic Science and Engineering 13, 74(1969).

The problem of timing of release has been addressed through the use of timing groups such as described in U.S. Pat. Nos. 4,248,962, 4,409,323 and 4,861,701. European Patent Applications 0 499 279 and 0 438 129 describe photographic compounds having a heterocyclic timing nucleus attached to a coupler moiety through an —O—C(O)— or —OCH<sub>2</sub>— group, or other group capable of releasing the heterocyclic timing nucleus by electron transfer down an unconjugated chain. However, the use of timing groups can create other problems. For example, many couplers have little flexibility in their rate of release of a PUG, or in their synthetic design, as they are limited by the presence of a particular first timing or linking group, particularly with regard to substituents on such groups. More importantly, though, some couplers exhibit poor stability when stored for prolonged periods under tropical conditions. Thus, they are of limited practical value in today's photographic industry.

Triazoles have been described for use as development inhibitors and have been utilized in DIR couplers, see for example U.S. Pat. Nos. 5,200,306, 5,360,709, 5,306,607, 5,380,633 and 5,270,157. However, the particularly useful compounds of this invention have not been utilized or suggested.

Therefore, a need has existed for a photographic coupler that is synthetically simple to manufacture; has the flexibility to work in a variety of situations; and that is stable when stored for prolonged periods, especially under tropical conditions. The coupler should be capable of releasing a devel-

opment inhibitor, thereby providing interlayer interimage effects and increased acutance for the image produced upon processing photographic material containing the coupler.

## SUMMARY OF THE INVENTION

This invention provides a photographic element comprising a support having situated thereon at least one silver halide emulsion layer, the element further containing an image modifying coupler which upon reaction with oxidized color developing agent during processing forms a dye, said image modifying coupler represented by the formula



wherein

COUP is a photographic coupler moiety;

T<sup>1</sup> is a timing or linking group;

R<sup>1</sup> and R<sup>2</sup> are independently selected from a halide atom, or an aliphatic, carbocyclic, heterocyclic, carbamoyl, sulfamoyl, carbonamido, sulfonamido, acyl, sulfo, nitro, cyano, amino, alkoxy, alkoxyalkyl, aryloxy, aryloxyalkyl, arylketo, alkylketo, thioalkoxy, thioalkoxyalkyl, thioaryloxy, or thioaryloxyalkyl group; and

n is selected from 0, 1 or 2. This invention more particularly provides a photographic element containing the above image modifying coupler wherein n is 0 and R<sup>2</sup> is represented by the formula



\*\* point of attachment to triazole moiety  
wherein;

Z is an aliphatic, carbocyclic, or heterocyclic group;

X is oxygen, sulfenate, sulfinate, sulfate, sulfur, sulfonyl, sulfinyl, selenium, selenonyl, seleninyl, or [—N(R<sup>4</sup>)—]; and

R<sup>3</sup> and R<sup>4</sup> are independently selected from hydrogen, or aliphatic, carbocyclic, heterocyclic groups, or acyl groups;

m is an integer from 0 to 10; and

t is 0,1 or 2. It further provides image modifying couplers as described above.

The image modifying couplers utilized in this invention provide improved interlayer interimage effects and acutance levels in the photographic elements in which they are contained. The new couplers are synthetically simple to manufacture and are much more stable than previously known photographic inhibitor releasing couplers containing a 1,2,3-triazole moiety. They are particularly stable during storage for prolonged periods at high temperatures. Further, the image modifying couplers are capable of and more preferably utilize direct release of 1,2,3-triazole inhibitors and they provide a wide range of reactivities depending upon the particular selection of the 1,2,3-triazole inhibitor and the substituents thereon. These couplers, unlike many other untimed or unlinked DIR couplers, can deliver a development inhibitor at a distance from the point at which oxidized color developing agent reacted with the coupler.

## DETAILED DESCRIPTION OF THE INVENTION

It has been surprisingly discovered that Development Inhibitor Releasing Couplers (DIRs) which comprise a tria-

zole inhibitor moiety which is attached to the coupler moiety through the 2'-nitrogen of the triazole moiety (as shown below) are more reactive than those attached to the 1'- or 3'-nitrogens of the triazole moiety. It has further been discovered that such DIRs, when comprising specific substituents on the triazole moiety, are very stable under prolonged storage conditions.

The imaging modifying couplers of this invention are represented by the formula



wherein COUP is a photographic coupler moiety and T<sup>1</sup> is a timing or linking group. While one of the main advantages of the image modifying couplers of this invention is that the coupler may be directly attached to the 1,2,3-triazole moiety, making the use of a timing or linking group unnecessary, an indirect attachment through a timing or linking group may be utilized. More preferably the attachment is direct. Therefore, n is selected from 0, 1 or 2 but is preferably 0. The 1'-, 2'- and 3'-nitrogen positions are as indicated. It will be appreciated that when R<sup>1</sup> and R<sup>2</sup> are the same the 1'-nitrogen and 3'-nitrogen positions are equivalent but that when R<sup>1</sup> and R<sup>2</sup> are not the same the 1'-nitrogen and 3'-nitrogen positions are not equivalent.

In the photographic coupler utilized in the present invention, the coupler moiety, as represented by COUP, can be any moiety that will react with oxidized color developing agent during processing to cleave the bond between T<sup>1</sup> and the coupler moiety or the triazole moiety and the coupler moiety. The coupler moiety as described herein includes conventional coupler moieties employed to yield both colorless and colored products upon reaction with oxidized color developing agents. Both types of coupler moieties are well known to those skilled in the photographic art and are exemplified in, for example, *Research Disclosure*, September 1994, Item 36544, all published by Kenneth Mason Publications, Ltd., Dudley Annex, 12a North Street, Emsworth, Hampshire PO10 7DQ, ENGLAND.

The coupler moiety can be ballasted or unballasted, and if unballasted, the dye formed upon oxidative coupling is capable of diffusing throughout, or being washed out of, the photographic element (sometimes known as a washout coupler). The coupler can be monomeric, or it can be part of a dimeric, oligomeric or polymeric coupler, in which case more than one triazole moiety can be contained in the coupler. The coupler can also form part of a bis compound in which the triazole moiety forms part of a link between two coupler moieties.

Representative coupler moieties suitable for use in the invention are as follows:

A. Couplers which form cyan dye upon reaction with oxidized color developing agent are described in such representative patents and publications as: U.S. Pat. Nos. 2,772,162; 2,895,826; 3,002,836; 3,034,892; 2,474,293; 2,423,730; 2,367,531; 3,041,236; 4,333,999 and "Farbkuppler-eine Literaturubersicht," published in Agfa Mitteilungen, Band III, pp. 156-175 (1961), all of which are incorporated herein by reference.

Preferably such cyan dye-forming couplers are phenols and naphthols.

B. Couplers which form magenta dye upon reaction with oxidized color developing agent are described in such rep-

resentative patents and publications as: U.S. Pat. Nos. 2,600,788; 2,369,489; 2,343,703; 2,311,082; 3,152,896; 3,519,429; 3,062,653; 2,908,573 and "Farbkuppler-eine Literaturubersicht," published in Agfa Mitteilungen, Band III, pp. 126-156 (1961), all of which are incorporated herein by reference.

Preferably such magenta dye-forming couplers are pyrazolones or pyrazolotriazoles.

C. Couplers which form yellow dye upon reaction with oxidized color developing agent are described in such representative patents and publications as: U.S. Pat. Nos. 2,875,057; 2,407,210; 3,265,506; 2,298,443; 3,048,194; 3,447,928 and "Farbkuppler-eine Literaturubersicht," published in Agfa Mitteilungen, Band III, pp. 112-126 (1961), all of which are incorporated herein by reference.

Preferably such yellow dye-forming couplers are acylacetamides, such as benzoylacetamides and pivaloylacetamides.

D. Couplers which form a colorless product upon reaction with oxidized color developing agent are described in such representative patents as: U.K. Patent No. 861,138; and U.S. Pat. Nos. 3,632,345; 3,928,041; 3,958,993 and 3,961,959, all of which are incorporated herein by reference.

Specific representative examples of coupler moieties suitable for use in the invention are as follows:



-continued



Formula (1G)



Formula (1H)



Formula (1I)



Formula (1J)



Formula (1K)

p in the above formulae can be 0 to 4; q can be 0 to 3; and r can be 0 to 5. The free bond in each of the coupler moieties described above represents the coupling site, which is the position to which the coupling-off group is linked. In the above formulae, R<sup>1a</sup>, R<sup>1b</sup>, R<sup>1c</sup>, R<sup>1d</sup>, R<sup>1e</sup>, R<sup>1f</sup>, R<sup>1g</sup>, R<sup>1h</sup>, R<sup>1i</sup>, R<sup>1j</sup>, or R<sup>1k</sup> may contain one or more solubilizing groups which will enable the coupler, upon reaction with oxidized color developing agent, to washout of the photographic element. Additionally, R<sup>1h</sup> and R<sup>1i</sup> can be a hydrogen. Such groups, and couplers containing them, are exemplified in U.S. Pat. Nos. 4,482,629; 5,026,628; 5,151,343; 5,250,398; and 5,250,399, which are incorporated herein by reference. Specifically preferred solubilizing groups are selected from a carboxyl, sulfo, carbonamido or hydroxyl group, or salt thereof. It is preferred that when a solubilizing group is present, the coupler moiety is also unballasted so that complete washing out of the dye can occur. By unballasted, it is meant that each R<sup>1a</sup> to R<sup>1k</sup> contain no more than 20 carbon atoms, preferably no more than 12 carbon atoms, and optimally no more than 8 carbon atoms.

R<sup>1a</sup> to R<sup>1k</sup>, p, q and r in formulae (1A) to (1K) are set forth in more detail as follows. Each of R<sup>1a</sup> to R<sup>1k</sup> is independently selected from the group consisting of a substituted or unsubstituted aliphatic, carbocyclic or heterocyclic group. Aliphatic, carbocyclic, and heterocyclic groups as used herein and elsewhere in this specification are defined in accordance with the definitions set forth in Grant and Hackh's *Chemical Dictionary*, fifth ed., McGraw-Hill 1987, and are in accordance with general rules of chemical nomenclature. The following descriptions of exemplary aliphatic,

carbocyclic and heterocyclic groups are intended to be utilized throughout this specification unless specifically noted otherwise.

5 Exemplary aliphatic groups include alkyl, alkene, and alkyne groups, particularly those having 1 to 25 carbon atoms. Examples of useful groups include methyl, ethyl, propyl, butyl, pentyl, hexyl, octyl, nonyl, decyl, dodecyl, hexadecyl, octadecyl, isopropyl, t-butyl, butenyl, pentenyl, hexenyl, octenyl, dodecenyl, propynyl, butynyl, pentynyl, hexynyl, and octynyl.

10 Exemplary carbocyclic groups (which include aryl groups) are those having a cyclic portion of 4 to 10 carbon atoms. Examples of useful groups include phenyl, tolyl, naphthyl, cyclohexyl, cyclopentyl, cyclohexenyl, cycloheptatrienyl, cyclooctatrienyl, cyclononatrienyl, cyclopentenyl, anilinyl, and anisidinyl.

15 Exemplary heterocyclic (which include heteroaryl groups) groups are those in which the cyclic portion has 5 to 10 atoms. Examples of useful groups include pyrrolyl, furyl, tetrahydrofuryl, pyridyl, picolinyl, piperidinyl, morpholinyl, thiadiazolyl, thiatriazolyl, benzothiazolyl, benzoxazolyl, benzimidazolyl, benzoselenazolyl, indazolyl, quinolyl, quinaldiny, pyrrolidinyl, thiophenyl, oxazolyl, thiazolyl, imidazolyl, selenazolyl, tellurazolyl, triazolyl, tetrazolyl, 20 oxadiazolyl, thietyl, pryanyl, chromenyl, isothiazolyl, isoxazolyl, pyrazinyl, pyrimidinyl, pyridazinyl, indolyl, purinyl, isoquinolyl, quinoxaliny, and quinazoliny. Preferred heteroatoms are nitrogen, oxygen, and sulfur.

25 35 It is understood throughout this specification and claims that any reference to a substituent by the identification of a group or a ring containing a substitutable hydrogen (e.g., alkyl, amine, aryl, alkoxy, heterocyclic, etc.), unless otherwise specifically described as being unsubstituted or as being substituted with only certain substituents, shall encompass not only the substituent's unsubstituted form but also its form substituted with any substituents which do not negate the advantages of this invention. Also, reference to 30 heterocyclic groups includes attachment at any position on the heterocycle. The term lower alkyl used herein means 1 to 5 carbon atoms. The term aryl or heterocyclic group or ring, unless otherwise indicated, includes bicyclic or other fused rings. Groups suitable for substitution, which may 35 themselves be substituted, include, but are not limited to, alkyl groups (for example, methyl, ethyl, hexyl), fluoroalkyl groups (for example, trifluoromethyl), alkoxy groups (for 40 example, methoxy, ethoxy, octyloxy), aryl groups (for example, phenyl, naphthyl, tolyl), hydroxy groups, halogen groups, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), carbamoyl and carbonamido groups, ureido groups, sulfamoyl and sulfonamido groups, acyloxy groups (for example, acetoxy, benzoxy), carboxy groups, cyano groups, sulfo groups, nitro groups and amino groups.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 90



wherein \* denotes the coupling site to which T<sup>1</sup> is attached.

R<sup>9</sup> is selected from hydrogen, or an aliphatic, carbocyclic, or heterocyclic group. In one embodiment this is a wash-out coupler and R<sup>9</sup> is preferably hydrogen, an alkyl group containing 1 to 5 carbon atoms, an aryl group containing 6 to 10 carbon atoms or a heterocyclic group containing 4 to 8 carbon atoms. In another embodiment R<sup>9</sup> is a ballast group which may contain the above groups.

V is independently selected from an alkyl, heterocyclic, halo, carbamoyl, sulfamoyl, carbonamido, sulfonamido, keto, sulfo, nitro, hydroxyl, carboxyl, amino, alkoxy, alkoxy carbonyl, aryloxy, or arylthio, group; and preferably from an alkyl containing 1 to 5 carbon atoms or a carbamoyl, sulfamoyl, carbonamido, sulfonamido, sulfo, nitro, hydroxyl, carboxyl, amino, alkoxy or alkoxy carbonyl group. j is 0, 1, 2, 3, or 4, preferably 0 or 1.

Also preferred are coupler moieties represented by



wherein \* denotes the coupling site to which T<sup>1</sup> is attached.

R<sup>10</sup> is selected from an aliphatic, carbocyclic, or heterocyclic group; and preferably from an alkyl group containing 1 to 10 carbon atoms, an aryl group containing 6 to 10 carbon atoms or a heterocyclic group containing 4 to 10 atoms;

Y is independently selected from an alkyl, heterocyclic, halo, carbamoyl, sulfamoyl, carbonamido, sulfonamido, keto, sulfo, nitro, hydroxyl, carboxyl, amino, alkoxy, alkoxy carbonyl, aryloxy or arylthio group. In one embodiment the coupler is a wash-out coupler and Y is preferably an alkyl group containing 1 to 5 carbon atoms, carbamoyl, sulfamoyl, carbonamido, sulfonamido, sulfo, nitro, hydroxyl, carboxyl, amino, alkoxy or alkoxy carbonyl group. p is 0, 1, 2, 3, or 4, preferably 1 or 2. In a more preferred embodiment Y is a ballast group which may contain the above groups.

Other preferred coupler moieties are represented by



wherein \* denotes the coupling site to which T<sup>1</sup> is attached.

R<sup>13</sup> and R<sup>14</sup> are independently selected from a hydrogen atom, or an aliphatic, carbocyclic, heterocyclic, carbamoyl, sulfamoyl, carbonamido, sulfonamido, acyl, alkylsulfonyl,

arylsulfonyl, alkylketo, arylketo, alkoxy carbonyl, aryloxy carbonyl, nitro, cyano, amino, alkoxy, alkoxy alkyl, aryloxy, aryloxy alkyl, thioalkoxy, thioalkoxy alkyl, thioaryloxy, or thioaryloxy alkyl group.

When R<sup>14</sup> is an amino group, preferred couplers are represented by



wherein R<sup>15</sup> an aliphatic, carbocyclic, or heterocyclic group.

In the above image modifying couplers R<sup>1</sup> and R<sup>2</sup> are independently selected from a halide or hydrogen atom, or an aliphatic, carbocyclic, heterocyclic, carbamoyl, sulfamoyl, carbonamido, sulfonamido, acyl, sulfo, nitro, cyano, amino, alkoxy, alkoxy alkyl, aryloxy, aryloxy alkyl, thioalkoxy, thioalkoxy alkyl, thioaryloxy, or thioaryloxy alkyl group or R<sup>1</sup> and R<sup>2</sup> may form a carbocyclic or heterocyclic ring. R<sup>1</sup> and R<sup>2</sup> may be the same or different. When they are different preferably R<sup>1</sup> or R<sup>2</sup> is a halide atom or an alkyl or carbocyclic group and the other is as defined below. In one suitable embodiment R<sup>1</sup> or R<sup>2</sup> is a carbocyclic group having 6 to 10 carbon atoms, and is preferably an aryl group.

Preferably R<sup>1</sup> and R<sup>2</sup> are independently represented by the formula



wherein \*\* represents the point of attachment to the triazole moiety. Z is selected from an aliphatic, carbocyclic, or heterocyclic group. m is an integer from 0 to 10 and more preferably m is 0 or 1. X is oxygen [-O-], sulfenate [-O-S-], sulfinate [-O-S(O)-], sulfate [-O-SO<sub>2</sub>-], sulfur [-S-], sulfonyl [-SO<sub>2</sub>-], sulfinyl [-S(O)-], selenium [-Se-], selenonyl [-SeO<sub>2</sub>-], seleninyl [-Se(O)-], or [-N(R<sup>4</sup>)-]; and t is 0, 1 or 2. Preferably X is oxygen, sulfur or [-N(R<sup>4</sup>)-]. R<sup>3</sup> and R<sup>4</sup> are independently selected from hydrogen, or aliphatic, carbocyclic, heterocyclic groups, or acyl groups. Preferably R<sup>3</sup> is an aliphatic group of 1 to 25 carbons, a carbocyclic group of 6 to 10 carbon atoms or a heterocyclic group of 5 to 10 atoms, particularly when t is 0. If R<sup>3</sup> is a heterocyclic group it may link through a heteroatom or a carbon atom. In one suitable embodiment R<sup>3</sup> is



wherein \*\*\*\* represents the point of attachment to \*\*-(Z)\_m-(X)\_t-\*\*\*\*

R<sup>7</sup> is an aliphatic, carbocyclic, heterocyclic, carbamoyl, sulfamoyl, carbonamido, sulfonamido, halogen, acyl, sulfo, nitro, cyano, amino, alkoxy, alkoxy alkyl, aryloxy, aryloxy alkyl, thioalkoxy, thioalkoxy alkyl, thioaryloxy, or thioaryloxy alkyl group; and s is an integer from 0 to 5.

In one embodiment X is oxygen or [-N(R<sup>4</sup>)-] and R<sup>3</sup> is an aliphatic, or carbocyclic group. In another suitable embodiment X is sulfur and R<sup>3</sup> is a heterocyclic group. In a further suitable embodiment X is oxygen and R<sup>3</sup> is an acyl group. Alternatively t may be 0.

In one preferred embodiment Z is represented by the formula



wherein \*\*\* represents the point of attachment to -(X)<sub>z</sub>R<sup>3</sup>. m is preferably 1 or 0. R<sup>5</sup> and R<sup>6</sup> are independently selected from hydrogen, or aliphatic, carbocyclic, or heterocyclic groups, or R<sup>1</sup>, R<sup>3</sup>, R<sup>4</sup>, R<sup>5</sup> and R<sup>6</sup> may be bonded together in pairs to form a 5 to 8 membered ring. Preferably R<sup>5</sup> and R<sup>6</sup> are hydrogen or a lower alkyl group. Again, in a suitable embodiment X is oxygen and R<sup>3</sup> is an acyl group or X is sulfur and R<sup>3</sup> is a heterocyclic group.

T<sup>1</sup>, if optionally utilized, can be any timing or linking group known in the art, for instance those described below and in U.S. Pat. Nos. 4,248,962; 4,409,323; 4,421,845; 4,857,447; 4,861,701; 4,864,604; 4,886,736; 4,891,304; 5,034,311; 5,055,385; 5,190,846; and European Patent Application 0 167 168, all of which are incorporated herein by reference. Thus, it may be a timing or linking group which functions by a nucleophilic displacement reaction (of the type described in, for example U.S. Pat. No. 4,248,962) or electron transfer down a conjugated chain (of the type described in, for example, U.S. Pat. No. 4,861,701). It may also be a timing or linking group which functions by electron transfer down an unconjugated chain. These last groups are known in the art under various names. Often they have been referred to as groups capable of utilizing a hemiacetal or iminoketal cleavage reaction or groups capable of utilizing a cleavage reaction due to ester hydrolysis. Regardless of their label, though, their mechanism is that of electron transfer down an unconjugated chain which results, typically, in a relatively fast decomposition and the production of carbon dioxide, formaldehyde or other low molecular weight by-products. Such groups are exemplified specifically in European Patent Application 0 464 612 and 0 523 451, both of which are incorporated herein by reference.

The image modifying couplers can be incorporated in photographic elements by means and processes known in the photographic art. Photographic elements in which the image modifying couplers are incorporated can be simple elements comprising a support and a single silver halide emulsion layer or multilayer, multicolor elements. The couplers can be incorporated in at least one of the light sensitive silver halide emulsion layers. The couplers may also be incorporated in a non-imaging layer or interlayer. The couplers may be contained in more than one layer, including in both imaging and non-imaging layers. In one embodiment the couplers are contained in an interlayer between a light sensitive layer and another light or non-light sensitive layer, such as an adjacent layer, where they will come into reactive association with oxidized color developing agent which has developed silver halide in the emulsion layer. By "in reactive association with" it is meant that the couplers can react or interact with, or come in contact with the developing agent.

The silver halide emulsion layer can contain or have associated with it other photographic couplers such as development inhibitor releasing couplers, including anchemically assisted development inhibitor releasing couplers, development agent releasing couplers, bleach inhibitor releasing couplers, electron transfer agent releasing couplers, development inhibiting redox releasing couplers, bleach accelerating releasing couplers, dye-forming couplers, colored masking couplers, and/or competing couplers. These other photographic couplers can form dyes of any color and hue or dyes which can wash out of the element

during processing. Additionally, the silver halide emulsion layers and other layers of the photographic element can contain addenda conventionally contained in such layers.

Atypical multilayer, multicolor photographic element can 5 comprise, preferably in the following order, a support having thereon a red-sensitive silver halide emulsion unit having associated therewith a cyan image dye forming coupler, a green-sensitive silver halide emulsion unit having associated therewith a magenta image dye forming coupler and a 10 blue-sensitive silver halide emulsion unit having associated therewith a yellow image dye forming coupler, at least one of the silver halide emulsion units or another layer having associated therewith an image modifying coupler as described above. Each silver halide emulsion unit can be 15 composed of one or more layers and the various units and layers can be arranged in different locations with respect to one another.

The silver halide emulsions can contain grains of any size and morphology. Thus, the grains may take the form of 20 cubes, octahedrons, cubo-octahedrons, or any of the other naturally occurring morphologies of cubic lattice type silver halide grains. Further, the grains may be irregular such as spherical grains or tabular grains. The light sensitive silver halide emulsions can include coarse, regular or fine grain 25 silver halide crystals or mixtures thereof, in a hydrophobic colloid, such as gelatin. The crystals can be comprised of any silver halide content, including silver chloride, silver bromide, silver bromoiodide, silver chlorobromide, silver chloroiodide, silver chlorobromoiodide and mixtures 30 thereof. The emulsions can be negative-working or positive-working emulsions and can be incorporated into negative or reversal elements as in U.S. Pat. No. 5,411,839, as well as other types of elements known in the art. They can form latent images predominantly on the surface of the silver halide grains or predominantly on the interior of the silver 35 halide grains. They can be chemically and spectrally sensitized by methods known in the art.

The silver halide photographic elements may also contain a transparent magnetic recording layer such as a layer 40 containing magnetic particles on the underside of a transparent support, as described in *Research Disclosure*, November 1992, Item 34390 published by Kenneth Mason Publications, Ltd., Dudley Annex, 12a North Street, Emsworth, Hampshire PO10 7DQ, ENGLAND. Typically, 45 the element will have a total thickness (excluding the support) of from about 5 to about 30 microns. Further, the photographic elements may have an annealed polyethylene naphthalate film base such as described in *Hatsumei Kyoushikai Koukai Gihou* No. 94-6023, published Mar. 15, 1994 50 (Patent Office of Japan and Library of Congress of Japan) and may be utilized in a small format system, such as described in *Research Disclosure*, June 1994, Item 36230 published by Kenneth Mason Publications, Ltd., Dudley Annex, 12a North Street, Emsworth, Hampshire PO10 7DQ, ENGLAND, and such as the Advanced Photo System, particularly the Kodak ADVANTIX films or cameras.

In the following Table, reference will be made to (1) *Research Disclosure*, December 1978, Item 17643, (2) *Research Disclosure*, December 1989, Item 308119, and (3) 60 *Research Disclosure*, September 1994, Item 36544, all published by Kenneth Mason Publications, Ltd., Dudley Annex, 12a North Street, Emsworth, Hampshire PO10 7DQ, ENGLAND, the disclosures of which are incorporated herein by reference. The Table and the references cited in the 65 Table are to be read as describing particular components suitable for use in the elements of the invention. The Table and its cited references also describe suitable ways of

preparing, exposing, processing and manipulating the elements, and the images contained therein. Photographic elements and methods of processing such elements particularly suitable for use with this invention are described in *Research Disclosure*, February 1995, Item 37038, published by Kenneth Mason Publications, Ltd., Dudley Annex, 12a North Street, Emsworth, Hampshire PO10 7DQ, ENGLAND, the disclosure of which is incorporated herein by reference.

| Reference | Section                        | Subject Matter                                                                                    |
|-----------|--------------------------------|---------------------------------------------------------------------------------------------------|
| 1         | I, II                          | Grain composition, morphology and preparation.                                                    |
| 2         | I, II, IX, X, XI, XII, XIV, XV | Emulsion preparation including hardeners, coating aids, addenda, etc.                             |
| 3         | I, II, III, IX A & B           | Chemical sensitization and spectral sensitization/desensitization                                 |
| 1         | III, IV                        | UV dyes, optical brighteners, luminescent dyes                                                    |
| 2         | IV, V                          |                                                                                                   |
| 1         | V                              |                                                                                                   |
| 2         | V                              |                                                                                                   |
| 3         | VI                             | Antifoggants and stabilizers                                                                      |
| 1         | VI                             |                                                                                                   |
| 2         | VII                            |                                                                                                   |
| 3         | VIII                           | Absorbing and scattering materials; Antistatic layers; matting agents                             |
| 1         | VIII, XIII, XVI                |                                                                                                   |
| 2         | VIII, IX C & D                 | Image-couplers and image-modifying couplers; Wash-out couplers; Dye stabilizers and hue modifiers |
| 3         | VII                            | Supports                                                                                          |
| 2         | VII                            |                                                                                                   |
| 3         | X                              |                                                                                                   |
| 1         | XVII                           | Specific layer arrangements                                                                       |
| 2         | XVII                           | Negative working emulsions;                                                                       |
| 3         | XV                             | Direct positive emulsions                                                                         |
| 3         | XI                             |                                                                                                   |
| 3         | XII, XIII                      | Exposure                                                                                          |
| 2         | XVIII                          |                                                                                                   |
| 3         | XVI                            |                                                                                                   |
| 1         | XIX, XX                        | Chemical processing;                                                                              |
| 2         | XIX, XX, XXII                  | Developing agents                                                                                 |
| 3         | XVIII, XIX, XX                 |                                                                                                   |
| 3         | XIV                            | Scanning and digital processing procedures                                                        |

The photographic elements can be incorporated into exposure structures intended for repeated use or exposure structures intended for limited use, variously referred to as single use cameras, lens with film, or photosensitive material package units.

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible dye image. Development is typically followed by the conventional steps of bleaching, fixing, or bleach-fixing, to remove silver or silver halide, washing, and drying.

The following examples illustrate the practice of the invention. They are intended to be illustrative, and should

not be construed as limiting the invention to the specific embodiments disclosed.

## EXAMPLES

### Example 1

The photographic elements were prepared by coating the following layers on a cellulose acetate film support (amounts of each component are indicated in mg/m<sup>2</sup>):

#### 15 Emulsion layer 1: (RECEIVER LAYER)

Gelatin-2420  
Red sensitized silver bromoiodide (as Ag)-1615  
Magenta image coupler (Ma-1)-557 dispersed in trityl phosphate.

#### 20 Interlayer

Gelatin-860  
Didodecylhydroquinone-113

#### 25 Emulsion layer 2: (CAUSER LAYER)

Gelatin-2690  
Green sensitized silver bromoiodide (as Ag)-1615  
30 Yellow image coupler (Ye-1)-694 dispersed in dibutyl phthalate  
DIR coupler of Tables 1 and 2 dispersed in trityl phosphate.

#### 35 Protective Overcoat

Gelatin-5380  
Bisvinylsulfonylmethyl ether at 2% total gelatin.

#### 40 The structures of the couplers utilized in the Examples are as follows:

##### Magenta Image Coupler, Ma-1:



**13**

-continued

Yellow Image Coupler, Ye-1:



Yellow DIR Coupler, D-1:



Yellow DIR Coupler, D-2:



Yellow DIR Coupler, I-1:

**14**

-continued

Yellow DIR Coupler, I-2:



Yellow DIR Coupler, I-3:



Yellow DIR Coupler, I-4:



Yellow DIR Coupler, I-5:



I-2

I-3

I-4

I-5

**15**

-continued

Yellow DIR Coupler, I-6:



Yellow DIR Coupler, I-7:



Yellow DIR Coupler, I-8:



Yellow DIR Coupler, I-9:

**16**

-continued

Yellow DIR Coupler, I-10:



-continued

## Magenta DIR Coupler, I-14:



### Magenta DIR Coupler, I-15:



## Magenta DIR Coupler, I-16:



Strips of each element were exposed to a green or white light through a graduated density step tablet, or through a 35% modulation fringe chart for sharpness measurements, and then developed for 3.25 minutes at 38° C. in the following color developer. Development was then stopped, and the elements were washed, bleached, fixed, and dried.

## Color Developer

|      |    |                                                                   |         |
|------|----|-------------------------------------------------------------------|---------|
| I-14 | 5  | Distilled water                                                   | 800 mL  |
|      |    | Sodium Sulfite, anhydrous                                         | 0.38 g  |
|      |    | CD-4 (color developer)*                                           | 4.52 g  |
|      |    | Potassium Carbonate, anhyd.                                       | 34.3 g  |
|      |    | Potassium Bicarbonate                                             | 2.32 g  |
|      |    | Sodium Bromide                                                    | 1.31 g  |
|      |    | Potassium Iodide                                                  | 1.20 mg |
|      | 10 | Hydroxylamine Sulfate                                             | 2.41 g  |
|      |    | Diethylenetriaminepentacetic acid,<br>pentasodium salt 40% Soln.) | 8.43 g  |
|      |    | Distilled water                                                   | to 1L   |
|      |    | Adjust pH to 10.0                                                 |         |

\*CD-4 is a KODAK color developer in which the active component is 4-amino-3-methyl-N-ethyl-N-beta-hydroxy-ethylaniline sulfate.

Photographic effects were determined as follows: To determine acutance(AMT), a series of elements as described above containing no DIR coupler or varying levels of DIR coupler were exposed with green light. The contrast ( $\gamma$ ) along the straight line portion of each elements'  $D \log H$  curve was measured. A plot of  $\log(\gamma)$  versus amount of DIR coupler ( $\mu$ moles) was made for each element (each element containing a different DIR coupler). From these plots, the amount of DIR coupler needed to achieve  $\log(0.7\gamma_0)$  was read, where  $\gamma_0$  represented the contrast of the element containing no DIR coupler. This value was recorded in Table 1 as Level<sup>\*</sup> (\* amount of DIR coupler need to reduce the contrast by 30%). In the same experiment, a plot of acutance versus  $\log(\gamma)$  was made for each element and from this plot the acutance at position  $\log(0.7\gamma_0)$  was read. These acutance values are shown in Table 1.

Acutance, as measured by AMT values and recorded in Table 1, are calculated using the following formula in which the cascaded area under the system modulation curve is shown in equation (21.104) on page 629 of the "Theory of the Photographic Process," 4th Edition, 1977, edited by T.

35 H. James:  $AMT = 100 + 66 \log[\text{cascaded area}/2.6696M]$   
 wherein the magnification factor M is 3.8 for the 35 mm  
 40  $AMT = 100 + 66 \log[100 \times 3.8] = 100 + 66 \log 380 = 100 + 66 \times 2.26 = 144$

40 system AMT. The use of CMT acutance is described by R. G. Gendron in "An Improved Objective Method of Rating Picture Sharpness: CMT acutance" in the Journal of SMPTE, Vol. 82, pages 1009-12, (1973). AMT is a further modification of CMT useful for evaluating systems which include the viewing of a positive print made from a negative.

45 Interlayer interimage effects representing the degree of color correction capable of being obtained by practice of the invention were evaluated after the same series of photographic elements were exposed to a white light. The log of the causer contrast ( $\gamma_c$ ) and the log of the receiver contrast ( $\gamma_r$ ) were read for each of the DIR levels in the elements and a plot of  $\log(\gamma_c)$  versus  $\log(\gamma_r)$  was made. From this plot,  $(\gamma_r)$  was determined at  $\log(0.7\gamma_c)$ , where  $\log(0.7\gamma_c)$  was measured along the causer axis in the plot. The ratio  $(\gamma_c)/(\gamma_r)$  was recorded in Table 1 as Interlayer Interimage.

TABLE 1

|    |             | Level <sup>*</sup><br>( $\mu\text{m}^2$ ) | Interlayer<br>Interimage<br>( $\gamma_c/\gamma_t$ ) | Accutance<br>(35 mm/causer) |
|----|-------------|-------------------------------------------|-----------------------------------------------------|-----------------------------|
| 55 | DIR Coupler |                                           |                                                     |                             |
|    | D-1         | 117.7                                     | 0.68                                                | 91.4                        |
|    | I-1         | 288.9                                     | 1.35                                                | 92.4                        |
|    | I-2         | 230.1                                     | 0.95                                                | 93.0                        |
|    | I-3         | 85.6                                      | 0.72                                                | 92.4                        |
|    | I-4         | 160.5                                     | 0.82                                                | 93.0                        |
|    | I-6         | 74.9                                      | 0.61                                                | 92.0                        |

\*Amount of DIR coupler coated that is needed to reduce contrast 30%

65 It can be seen from Table 1 that the couplers of the invention give acceptance and/or interlayer interimage effects superior to those of the control coupler D-1.

## 19

## Example 2

The photographic elements of Example 2 were prepared and processed, and the results measured and calculated, as described for Example 1. The results are shown in Table 2.

TABLE 2

| DIR Coupler | Level*<br>( $\mu\text{m}^2$ ) | Interlayer<br>Interimage<br>( $\gamma_c/\gamma_i$ ) | Accutance<br>(35 mm/causer) |
|-------------|-------------------------------|-----------------------------------------------------|-----------------------------|
| D-1         | 107                           | 0.659                                               | 92.0                        |
| D-2         | 69.6                          | 0.659                                               | 92.8                        |
| I-5         | 53.5                          | 0.596                                               | 92.0                        |
| I-6         | 85.6                          | 0.757                                               | 92.8                        |
| I-8         | 112.4                         | 0.659                                               | 92.8                        |
| I-9         | 37.5                          | 0.560                                               | 91.0                        |
| I-10        | 107.0                         | 0.830                                               | 94.0                        |
| I-12        | 69.6                          | 0.629                                               | 92.0                        |
| I-13        | 128.4                         | 0.830                                               | 94.0                        |

\*Amount of DIR coupler coated that is needed to reduce contrast 30%

It can be seen from Table 2 that the couplers of the invention give accutance, interlayer interimage effects and/or activity (amount of DIR coated), superior to those of control couplers D-1 and D-2.

## Example 3

Strips of the photographic elements of Examples 1 and 2 were stored and incubated for 4 weeks at 49° C. and 50% relative humidity. The stability of the couplers utilized in the invention and the comparative couplers is shown in Table 3 as % loss. Specifically, % loss was determined by extracting the coupler from the elements after incubation and comparing the amount (weight) of coupler extracted with the amount (weight) extracted from similar elements that were not incubated. Extraction was performed by methods known in the art and measurements of coupler amounts were made by HPLC analysis.

| DIR Coupler | % Loss** | DIR Coupler | % Loss** |
|-------------|----------|-------------|----------|
| D-1         | 1        | I-8         | 0        |
| D-2         | 28       | I-9         | 4        |
| I-1         | 5        | I-10        | 3        |
| I-2         | 3        | I-12        | 0        |
| I-3         | 5        | I-13        | 13       |
| I-4         | 9        | I-14        | 6        |
| I-5         | 8        | I-15        | 4        |
| I-6         | 5        | I-16        | 1        |
| I-7         | 6        |             |          |

\*\*% loss of the coupler from the photographic elements after 4 weeks at 49° C. and 50% relative humidity.

It can be seen from Table 3 that the couplers utilized in this invention have superior stability when stored under tropical conditions. It can also be seen from Tables 1, 2 and 3 that while couplers D-1 and D-2 show single advantages such as having either good accutance or good stability; the couplers of the invention show multiple advantages, i.e. they demonstrate good accutance, interimage effects and stability.

## Example 4

The photographic element was prepared by coating the following layers on a film support with a grey silver antihalation layer (amounts of each component are indicated in  $\text{mg}/\text{m}^2$ ):

Emulsion Layer 1; (RECEIVER LAYER) Gelatin-2688. Red sensitized silver bromoiodide (as Ag)-806. Magenta

## 20

Image Coupler (Ma-1):tritoly phosphate:Stabilizer (ST-1), in the ratio 1.0:0.8:0.2 (respectively)-430  
INTERLAYER LAYER Gelatine-860. Interlayer Scavenger (S-1)-54.

Emulsion Layer 2: (CAUSER LAYER) Gelatin-2688. Green sensitized silver bromoiodide (as Ag)-806. Yellow Image Coupler (Ye-1)-860, dispersed in tritoly phosphate (1:0.5), and DIR Couplers I-17, I-18, I-19, I-20 and I-23 of Table 4 dispersed in tritoly phosphate.

PROTECTIVE OVERCOAT Gelatin-5375. Bisvinylsulfonylmethyl ether-281.

The elements were subjected to a green exposure and a neutral exposure and processed by bleaching and fixing as described in Example 1. The blue contrast was read for the green exposure (B of G), and green contrast read for the neutral exposure (G of N). The results are shown in Table 4.

TABLE 4

| Entry No.      | DIR Coupler | Level (mmoles/sq. m) | % Contrast Reduction (B of G) <sup>1</sup> | % Contrast Reduction (G of N) <sup>2</sup> |
|----------------|-------------|----------------------|--------------------------------------------|--------------------------------------------|
| 1<br>(control) | none        | 0                    | 0                                          | 0                                          |
| 2<br>(check)   | D-1         | 54                   | -22                                        | -4                                         |
|                |             | 108                  | -27                                        | -10                                        |
|                |             | 161                  | -34                                        | -21                                        |
| 3              | I-17        | 54                   | -13                                        | -17                                        |
|                |             | 108                  | -18                                        | -27                                        |
|                |             | 161                  | -22                                        | -36                                        |
| 4              | I-18        | 54                   | -26                                        | -21                                        |
|                |             | 108                  | -43                                        | -39                                        |
|                |             | 161                  | -60                                        | -40                                        |
| 5              | I-19        | 54                   | -54                                        | -29                                        |
|                |             | 108                  | -69                                        | -43                                        |
|                |             | 161                  | -74                                        | -49                                        |
| 6              | I-20        | 54                   | -17                                        | -22                                        |
|                |             | 108                  | -27                                        | -36                                        |
|                |             | 161                  | -41                                        | -43                                        |
| 7              | I-23        | 54                   | -29                                        | -18                                        |
|                |             | 108                  | -42                                        | -32                                        |
|                |             | 161                  | -49                                        | -39                                        |

<sup>1</sup>Blue contrast obtained from a green only exposure.

<sup>2</sup>Green contrast obtained from a neutral exposure. This is a measure of the Interlayer Interimage of the element.

## Example 5

The photographic element was prepared by coating the following layers on a film support with a grey silver antihalation layer (amounts of each component are indicated in  $\text{mg}/\text{m}^2$ ):

Emulsion Layer 1; (RECEIVER LAYER) Gelatin-2688. Red sensitized silver bromoiodide (as Ag)-806. BAR Coupler (B-1)-5. DIR Coupler (D-3)-22. Cyan Image Coupler (C-1)-753, dispersed in dibutylphthalate  
INTERLAYER LAYER Gelatine-860. Interlayer Scavenger (S-1)-54.

Emulsion Layer 2; (CAUSER LAYER) Gelatin-2688. Green sensitized silver bromoiodide (as Ag)-806. Magenta Image Coupler (Ma-1):tritoly phosphate:Stabilizer (ST-1) in the ratio 1.0:0.8:0.2 (respectively)-430 and DIR Couplers I-25 and I-27 of Table 5 dispersed in tritoly phosphate.

PROTECTIVE OVERCOAT Gelatin-5375. Bisvinylsulfonylmethyl ether-281.

The elements were subjected to a green exposure and a neutral exposure and processed by bleaching and fixing as described in Example 1. The green contrast was read for the green exposure (G of G), and red contrast read for the neutral exposure (R of N).

The results of the experiment are shown in Table 5.

TABLE 5

| Entry No.   | DIR Coupler | Level (mmoles/sq. m) | % Contrast Reduction (G of G) <sup>1</sup> Causer Layer | % Contrast Reduction (R of N) <sup>2</sup> Receiver Layer |
|-------------|-------------|----------------------|---------------------------------------------------------|-----------------------------------------------------------|
| 8 (control) | none        | 0                    | 0                                                       | 0                                                         |
| 9           | I-25        | 54                   | -32                                                     | -32                                                       |
|             |             | 108                  | -45                                                     | -38                                                       |
|             |             | 161                  | -49                                                     | -40                                                       |
| 10          | I-27        | 54                   | -42                                                     | -22                                                       |
|             |             | 108                  | -52                                                     | -29                                                       |

<sup>1</sup>Green contrast obtained from a green only exposure.

<sup>2</sup>Red contrast obtained from a neutral exposure. This is a measure of the Interlayer Interimage of the element.

It can be seen from Tables 4 and 5 that in comparison to the check D-1; the compounds of the invention are very effective at reducing the contrast in not only the causer layer, but also in the receiver layer.

The structures of the couplers and compounds utilized in Examples 4 and 5 are as follows:

Stabilizer, ST-1:



Interlayer Scavenger, S-1:



Cyan Image Coupler, C-1:



-continued

BAR Coupler, B-1:



DIR Coupler, D-3



DIR Coupler I-17



**23**

-continued

DIR Coupler I-18



DIR Coupler I-19



DIR Coupler I-20



DIR Coupler I-21

**24**

-continued

DIR Coupler I-22



DIR Coupler I-23



DIR Coupler I-24



**25**

-continued

DIR Coupler I-25

**26**

-continued

DIR Coupler I-28



DIR Coupler I-26



DIR Coupler I-29



DIR Coupler I-27



The invention has been described in detail with particular reference to preferred embodiments thereof, but it will be understood that variations and modifications can be effected within the spirit and scope of the invention.

What is claimed is:

1. A photographic element comprising a support having situated thereon at least one silver halide emulsion layer, the element further containing an image modifying coupler which upon reaction with oxidized color developing agent during processing forms a dye, said image modifying coupler represented by the formula



55

60

wherein

COUP is a photographic coupler moiety;

T<sup>1</sup> is a timing or linking group;

R<sup>1</sup> and R<sup>2</sup> are independently selected from a halide atom, or an aliphatic, carbocyclic, heterocyclic, carbamoyl, sulfamoyl, carbonamido, sulfonamido, acyl, sulfo, nitro, cyano, amino, alkoxy, alkoxyalkyl, aryloxy, aryloxyalkyl, thioalkoxy, thioalkoxyalkyl, thioaryloxy, or thioaryloxyalkyl group; and

n is selected from 0, 1 or 2.

2. The photographic element of claim 1 wherein R<sup>1</sup> and R<sup>2</sup> are independently represented by the formula:



\*\* point of attachment to triazole moiety  
wherein:

Z is an aliphatic, carbocyclic, or heterocyclic group;

X is oxygen, sulfenate, sulfinate, sulfate, sulfur, sulfonyl, sulfinyl, selenium, selenonyl, seleninyl, or [—N(R<sup>4</sup>)—]; and

R<sup>3</sup> and R<sup>4</sup> are independently selected from hydrogen, or aliphatic, carbocyclic, heterocyclic groups, or acyl groups;

m is an integer from 0 to 10; and

t is 0, 1 or 2.

3. The photographic element of claim 2 wherein n is 0.

4. The photographic element of claim 3 wherein for at least one of R<sup>1</sup> or R<sup>2</sup> t is 0, m is 0 and R<sup>3</sup> is an aliphatic or carbocyclic group.

5. The photographic element of claim 4 wherein R<sup>3</sup> is an aryl group.

6. The photographic element of claim 3 wherein for at least one of R<sup>1</sup> or R<sup>2</sup> X is oxygen, sulfur or nitrogen.

7. The photographic element of claim 6 wherein for at least one of R<sup>1</sup> or R<sup>2</sup> X is oxygen or —N(R<sup>4</sup>)— and R<sup>3</sup> is an aliphatic, or carbocyclic group and R<sup>4</sup> is hydrogen or an aliphatic, carbocyclic, heterocyclic or acyl group.

8. The photographic element of claim 6 wherein for at least one of R<sup>1</sup> or R<sup>2</sup> X is sulfur and R<sup>3</sup> is a heterocyclic group.

9. The photographic element of claim 6 wherein for at least one of R<sup>1</sup> or R<sup>2</sup> X is oxygen and R<sup>3</sup> is an acyl group.

10. The photographic element of claim 3 wherein for at least one of R<sup>1</sup> or R<sup>2</sup> Z is represented by the formula



\*\*\* point of attachment to -(X)\_t-R<sup>3</sup>  
wherein

R<sup>5</sup> and R<sup>6</sup> are independently selected from hydrogen, or aliphatic, carbocyclic, or heterocyclic groups, or R<sup>1</sup>, R<sup>3</sup>, R<sup>4</sup>, R<sup>5</sup> and R<sup>6</sup> may be bonded together in pairs to form a 5 to 8 membered ring.

11. The photographic element of claim 3 wherein for at least one of R<sup>1</sup> or R<sup>2</sup> m is 0 or 1.

12. The photographic element of claim 10 wherein m is 0 or 1.

13. The photographic element of claim 10 wherein X is oxygen and R<sup>3</sup> is an acyl group.

14. The photographic element of claim 10 wherein X is sulfur and R<sup>3</sup> is a heterocyclic group.

15. The photographic element of claim 3 wherein for at least one of R<sup>1</sup> or R<sup>2</sup> t is 0.

16. The photographic element of claim 10 wherein R<sup>3</sup> is an aliphatic group of 1 to 25 carbons, a carbocyclic group of 6 to 10 carbon atoms or a heterocyclic group of 5 to 10 atoms.

17. The photographic element of claim 16 wherein R<sup>3</sup> is



\*\*\*\* represents the point of attachment to \*\*-(Z)\_m-(X)\_t-\*\*\*\*

wherein

R<sup>7</sup> is an aliphatic, carbocyclic, heterocyclic, carbamoyl, sulfamoyl, carbonamido, sulfonamido, halogen, acyl, sulfo, nitro, cyano, amino, alkoxy, alkoxyalkyl, aryloxy, aryloxyalkyl, thioalkoxy, thioalkoxyalkyl, thioaryloxy, or thioaryloxyalkyl group; and

s is an integer from 0 to 5.

18. The photographic element of claim 10 wherein t is 0.

19. The photographic element of claim 16 wherein t is 0.

20. The photographic element of claim 3 wherein the image modifying coupler is contained in a light-sensitive silver halide emulsion layer.

21. The photographic element of claim 3 wherein the image modifying coupler is located in an interlayer between two light-sensitive silver halide emulsion layers.

22. The photographic element of claim 20 wherein the silver halide emulsion layer contains a development inhibitor releasing coupler in addition to the image modifying coupler.

23. The photographic element of claim 22 wherein the development inhibitor releasing coupler is an anchimerically assisted development inhibitor releasing coupler.

24. The photographic element of claim 20 wherein the silver halide emulsion layer contains a bleach accelerator releasing coupler in addition to the image modifying coupler.

25. The photographic element of claim 1 comprising a support bearing

at least one red sensitive photographic silver halide emulsion layer comprising at least one cyan image dye-forming coupler;

at least one green sensitive photographic silver halide emulsion layer comprising at least one magenta image dye-forming coupler;

at least one blue sensitive photographic silver halide emulsion layer comprising at least one yellow image dye-forming coupler; and

wherein the image modifying compound is in reactive association with a light-sensitive photographic silver halide emulsion layer.

26. A photographic image modifying coupler represented by the formula



wherein

COUP is a photographic coupler moiety;

T<sup>1</sup> is a timing or linking group;

R<sup>1</sup> and R<sup>2</sup> are independently selected from a halide or hydrogen atom, or an aliphatic, carbocyclic, heterocyclic, carbamoyl, sulfamoyl, carbonamido, sulfonamido, acyl, sulfo, nitro, cyano, amino, alkoxy, alkoxyalkyl, aryloxy, aryloxyalkyl, thioalkoxy, thioalkoxyalkyl, thioaryloxy, or thioaryloxyalkyl group or R<sup>1</sup> and R<sup>2</sup> may form a carbocyclic or heterocyclic ring; and

n is 0, 1 or 2.

**27.** The photographic image modifying coupler of claim 26 wherein R<sup>1</sup> and R<sup>2</sup> are independently represented by the formula:



\*\* point of attachment to triazole moiety

wherein;

Z is an aliphatic, carbocyclic, or heterocyclic group;

X is oxygen, sulfenate, sulfinate, sulfate, sulfur, sulfonyl, sulfinyl, selenium, selenonyl, seleninyl, or [—N(R<sup>4</sup>)—]; and

R<sup>3</sup> and R<sup>4</sup> are independently selected from hydrogen, or aliphatic, carbocyclic, heterocyclic groups, or acyl group;

m is an integer from 0 to 10; and

t is 0, 1 or 2.

**28.** The photographic element of claim 2 wherein m is 0, X is sulfur, t is 1 and R<sup>3</sup> is a substituted aliphatic group.

**29.** The photographic element of claim 2 wherein m is 0, t is 0 and R<sup>3</sup> is a substituted aliphatic or substituted carbocyclic group.

**30.** The photographic element of claim 2 wherein said image modifying coupler is

DIR Coupler I-17



DIR Coupler I-18



DIR Coupler I-19



DIR Coupler I-20



**31**

-continued

DIR Coupler I-21



DIR Coupler I-22



DIR Coupler I-23



DIR Coupler I-24

**32**

-continued

DIR Coupler I-25



DIR Coupler I-26



DIR Coupler I-27



6,007,974

**33**

-continued

DIR Coupler I-28  
n-C<sub>11</sub>H<sub>23</sub>CONH



or



**34**

-continued

DIR Coupler I-29

n-C<sub>11</sub>H<sub>23</sub>CONH

5

10

15

20



\* \* \* \* \*